

Dec. 26, 1961

G. A. LYON

3,014,272

METHOD OF PREPARING METAL BLANKS

Filed Nov. 23, 1955

3 Sheets-Sheet 1



Fig-5



Fig-2



INVENTOR  
GEORGE ALBERT LYON

By Hill, Sherman, Moran, Gross & Simpson Atty's.

Dec. 26, 1961

G. A. LYON

3,014,272

METHOD OF PREPARING METAL BLANKS

Filed Nov. 23, 1955

3 Sheets-Sheet 2



INVENTOR  
GEORGE ALBERT LYON

By Hill, Sherman, Moran, Gross & Simpson Atty's.

Dec. 26, 1961

G. A. LYON

3,014,272

METHOD OF PREPARING METAL BLANKS

Filed Nov. 23, 1955

3 Sheets-Sheet 3



by Hill, Sherman, Moran, Gross & Simpson, Atty.

1

3,014,272

METHOD OF PREPARING METAL BLANKS  
 George Albert Lyon, Detroit, Mich., assignor to Lyon Incorporated, Detroit, Mich., a corporation of Delaware  
 Filed Nov. 23, 1955, Ser. No. 548,597  
 5 Claims. (Cl. 29—526.6)

The present invention relates to improvements in the preparation of metal blanks and more particularly concerns the preparation of ingot pieces for cupping and drawing into shell form.

In the manufacture of steel shells, and more especially such shells of substantial size, it is desirable as an economy measure to utilize material derived directly from cast ingots. However this presents the problem of removing the scale and other impurities, flutes, cracks, pits, and the like, present on the surfaces, and more particularly the longitudinal surfaces of the ingot pieces. It is highly desirable to have the ingot pieces as clean and presenting at the surfaces thereof as nearly pure steel without flaws as practicable.

It is accordingly an important object of the present invention to provide an improved method of cleaning up steel ingot pieces intended for eventual drawing fabrication.

Another object of the invention is to provide steel blanks derived from ingot pieces in a clean, substantially flawless condition so that steel shells drawn therefrom will be substantially uniform and free from undesirable imperfections.

A further object of the invention is to provide improved means for preparing ingot pieces for drawing into steel shells.

According to the general features of the present invention, there is provided a method of cleaning tapered ingot pieces which are of smaller outside diameter at one end relative to the opposite end, wherein axial compression is applied to each piece to a limited extent just sufficient for bulging the longitudinal wall thereof laterally accompanied by a component of additional lateral pressure thrust from the center outwardly at the smaller diameter end of the piece by pressing of a shallow substantially conical depression into the smaller diameter end of the piece, such depression having a substantial diameter relative to the diameter of the ingot piece, so as to displace material from the center of the smaller diameter end to compensate for the reduction in diameter of the piece toward that end and thus effect substantially uniform bulging of the originally smaller diameter longitudinal wall portion outwardly substantially to match the bulging diameter of the originally larger diameter end wall portion of the piece.

According to other general features of the invention, the bulged longitudinal wall material is trimmed off to substantially a predetermined wall perimeter to expose substantially flawless clean material of the piece about the entire longitudinal wall perimeter to afford a clean periphery on the piece.

Other objects, features and advantages of the present invention will be readily apparent from the following detailed description of certain preferred embodiments thereof taken in conjunction with the accompanying drawings in which:

FIGURE 1 is a more or less schematic vertical sectional elevational view through apparatus for scalping an ingot piece;

FIGURE 2 is a fragmentary horizontal sectional view taken substantially on the line II—II of FIGURE 1;

FIGURE 3 is a vertical sectional elevational view similar to FIGURE 1 but showing the apparatus in the relationship of the components in one phase of operation thereof on the ingot piece;

2

FIGURE 4 is a sectional elevational view similar to FIGURES 1 and 3 but showing the relationship of the components of the apparatus following a blank shaping and scalping operation;

5 FIGURE 5 is a fragmentary elevational view of an ingot with substantially straight tapering longitudinal walls, showing a piece partially severed for cleaning according to the present method and in the apparatus of FIGURES 1 through 4;

10 FIGURE 6 is an isometric view of a billet that may have been derived by reshaping a cleaned ingot piece;

15 FIGURE 7 is a more or less schematic view showing how either the cleaned ingot piece of FIGURE 4 or the billet of FIGURE 6 is adapted to be flattened into thin disk form preparatory to cupping the same and drawing into shell form; and

20 FIGURE 8 is a fragmentary vertical sectional elevational view showing a cupping die structure.

25 As cast at the mill steel ingots are generally several feet long and a foot or so in diameter. They may be generally straight sided or they may be fluted. In either event, they are tapered from one end toward the other.

30 For the purpose of preparing pieces of the ingots for drawing, the ingots are divided into pieces which are calculated as to length in relation to the taper to afford equal mass in each of the pieces or sections of the ingot. At the opposite ends of the pieces so separated from the ingot clean surfaces will be provided incident to the separation. It will be understood, of course, that all piping will be trimmed off, as well as the end face where there is no piping. Hence, it is necessary in order to provide a piece that is satisfactory for drawing to trim off or scalp the longitudinal periphery of each piece.

35 According to the present invention, scalping or cleaning up of the longitudinal surface of a billet piece 10 (FIGS. 1 and 2) which may be fluted as shown, is accomplished by compressing the piece axially to bulge the fluted perimeter free from the taper and to substantially crack and dislodge scale therefrom. Then the ingot piece 40 10 is smoothly and uniformly trimmed off.

45 Herein compressing and bulging and trimming of the ingot piece 10 are accomplished in a combination press and scalping die structure including a columnar supporting or anvil member 11 of cylindrical form, an opposing complementary pressure applying, ingot piece bulging punch member 12, and a scalping member 13. The anvil member 11 is supported upon a base structure 14 which may be a press bed. The upper end of the anvil member 11 is adapted to support the ingot piece 10 thereon and is preferably of a diameter to which the ingot piece is to be trimmed after it is bulged.

55 A cooperative relationship is provided whereby the bulging punch 12 is reciprocably guided by and within the scalping member 13. To this end the punch 12 is preferably cylindrical and the member 13 is preferably tubular and is provided with a longitudinal bore 15 within which the punch is slidable. By preference the diameter of the bore 15 is about the same as the diameter of the at least upper end portion of the anvil member 11 60 and equal to the diameter to which the ingot piece is to be trimmed.

65 About the mouth of the trimming die bore 15 is a shearing edge 17 of generally chisel point in cross-section but circular in shape with a generally frusto-conical surface 18 sloping upwardly and outwardly therefrom.

70 For receiving and stripping material trimmed off by the trim die member 13, a ring member 19 is provided about the anvil cylinder 11 and connected to the trimming die member 13 by rigid longitudinally extending connecting arms 20 of which there may be a pair at diametrically opposite sides. Between the arms 20, as well as between the ring 19 and the shearing end 17

of the member 13, ample access space to the compression space between the punch and anvil is afforded. The ring member 19 may also serve as a guide for assuring registration of the punch and die members.

In operation, the ingot piece 10 is placed upon the top of the anvil member 11 as shown in FIGURE 1. Then the punch member 12 is motivated to apply compressive force against the ingot piece toward the anvil member 11. This causes a shallow-taper, generally frusto-conical nose 21 on the pressure or thrust end of the punch 12 to be pressed centrally into the opposing surface of the ingot piece 10 to thereby cause greater lateral displacement of the material in the adjacent end portion of the ingot piece 10 to occur than in the opposite end portion, so as to compensate for taper of the longitudinal surface of the ingot piece which is disposed between the compression members with the smaller end of the taper directed toward the punch nose 21. The compressive force is applied until sufficient of the longitudinal surface of the ingot piece 10 has been bulged laterally into overhanging relation to the periphery of the anvil member 11, and beyond the diameter of the shearing edge 17 as shown in dash outline in FIGURE 1 and in full line in FIGURE 3. At the same time a central boss 22 of material at the opposite end face of the ingot piece 10, which may in part comprise a remainder of a connecting neck at which the piece was severed from the ingot, is pressed into a centering recess 23 in the supporting face of the anvil member 11. Thereby the ingot piece 10 is firmly centered against any possibility of shifting or skewing incident to pressure against the sides thereof as the shearing edge 17 is operated to scalp the longitudinal perimeter of the piece.

As thus bulged and firmly held between the anvil 11 and the punch 12, scalping of the longitudinal perimeter of the ingot piece is accomplished by driving of the trimming member 13 longitudinally relative to the punch and anvil and the slightly compressed and laterally bulged piece 10 held therebetween to scalp off the more or less irregular longitudinal perimeter substantially as shown in dash outline in FIGURE 3. As the trimming or scalping proceeds, the trimmed and cleaned longitudinal surface is received within the bore 15, and the chip C curls down under the tapered edge 18 until it is severed from the work piece and is deposited about the anvil 11 to which it may cling.

Following the trimming action, the trimming member 13 and the punch 12 are backed off successively from the trimmed ingot piece 10, the punch 12 serving as a stripper or hold-down in engagement with the trimmed ingot piece until the trimming member 13 has been backed off free from the ingot piece. The trimmed ingot piece 10 is then lifted from the anvil 11. If necessary the trimming member 13 may then be backed off further until the chip ring C has been stripped free from the anvil 11 or at least lifted clear of the anvil to facilitate removal of the chip.

At completion of the trimming or scalping operation, as shown in FIGURE 4, the now cleaned ingot piece 10 is removed and may, if it is to be stored for any length of time, be surface treated or coated to avoid oxidation or corrosion.

On the other hand, if it is desired to compact and reorient the grain of the clean piece 10, it may be heated and forged into a polygonal block such as a square block 25 as shown in FIGURE 6.

Instead of being fluted as shown in FIGURE 1, an ingot piece 10' (FIG. 5) may be derived from a straight sided tapered ingot I by cutting a separation 24 to the connecting neck 22', complete separation of the piece 10' is then effected by cracking the neck 22' as by driving a wedge into the severance cut or slot 24.

Preparation of the ingot pieces or billets is, of course, preliminary to transforming the shape thereof into a flattened blank B (FIGS. 7 and 8). By subjecting the cleaned piece to axial pressure to compress the same uni-

formly it is laterally spread or displaced and axially reduced in thickness until the desired flattened blank thickness is attained. Such flattening is preferably accomplished while the metal piece is at a good working heat such as 2000° F. to 2200° F.

Then, preferably while the disk is still hot it is placed in suitable trimming and cupping mechanism such as shown in FIGURE 8. This includes a combination trimming die and cupping die ring member 27 with which is cooperatively reciprocally related a trimming shear ring 28. Through this arrangement the blank B centered upon the cupping and shearing ring die 27 has the marginal portion thereof trimmed as indicated by the dotted circular line T in FIGURE 7. Then, while the trimmed blank B is held centered on the ring die member 27 following the trimming, a cupping punch 29 thrusts axially thereagainst to cup the blank as indicated in dash and dot dash lines in FIGURE 8. Following the cupping the blank is stripped free from the cupping punch 29 by strippers 30. The cupped blank B is ready to be drawn into elongated shell form.

It will be understood that modifications and variations may be effected without departing from the scope of the novel concepts of the present invention.

I claim as my invention:

1. In a method of cleaning tapered ingot pieces which are of smaller outside diameter at one end relative to the opposite end, applying axial compression to each piece to a limited extent just sufficient for bulging the longitudinal walls thereof laterally accompanied by a component of additional lateral pressure thrust from the center outwardly at the smaller diameter end of the piece so as to displace material from said center of the smaller diameter end to compensate for the reduction in diameter of the piece toward that end and thus effect substantially uniform bulging of the originally smaller diameter longitudinal wall portion outwardly substantially to match the bulging diameter of the originally larger diameter end wall portion, and then trimming off the bulged longitudinal wall material to substantially a predetermined wall perimeter to expose substantially flawless clean material of the pieces about the entire longitudinal wall perimeter to afford a clean periphery on the pieces, said additional lateral pressure thrust component being effected by pressing of a shallow substantially conical depression into the smaller diameter end of the piece in each instance, the depression having a substantial diameter relative to the diameter of the ingot piece.

2. In a method of reshaping the longitudinal wall of a tapered ingot piece preparatory to trimming the longitudinal wall wherein one end of the piece is of an originally smaller diameter than the opposite end, placing the ingot piece with its larger end on an anvil member having a diameter substantially the same as the diameter of the larger end of the piece, driving a shallow-taper generally frusto-conical punch nose having a substantial diameter relative to the diameter of the ingot centrally into the smaller diameter end of the piece and thereby pressing a shallow complementary frusto-conical depression into said smaller diameter end and thus displacing material of the piece from the smaller diameter end portion thereof downwardly and laterally and thereby bulging the longitudinal perimeter of the piece into substantially uniform shape and eliminating the taper thereof.

3. In a method of cleaning the longitudinal wall of a tapered ingot piece wherein one end of the piece is of an originally smaller diameter than the opposite end, placing the ingot piece with its larger end on an anvil member having a diameter substantially the same as the diameter of the larger end of the piece, driving a shallow-taper generally frusto-conical punch nose having a substantial diameter relative to the diameter of the ingot centrally into the smaller diameter end of the piece and thereby pressing a shallow complementary frusto-conical depression into said smaller diameter end and thus displacing material of the piece from the smaller diameter

end portion thereof downwardly and laterally and thereby bulging the longitudinal perimeter of the piece into substantially uniform shape and eliminating the taper thereof, and while holding the bulged piece on said anvil by said punch pressing into said depression, trimming off the bulged perimeter of the piece to expose clean material on the perimeter of the piece.

4. In a method of cleaning the longitudinal wall of a tapered ingot piece wherein one end of the piece is of an originally smaller diameter than the opposite end, placing the ingot piece with its larger end on an anvil member having a diameter substantially the same as the diameter of the larger end of the piece, driving a shallow-taper generally frusto-conical punch nose having a substantial diameter relative to the diameter of the ingot centrally into the smaller diameter end of the piece and thereby pressing a shallow complementary frusto-conical depression into said smaller diameter end and thus displacing material of the piece from the smaller diameter end portion thereof downwardly and laterally and thereby bulging the longitudinal perimeter of the piece into substantially uniform shape and eliminating the taper thereof, as an incident to pressing said depression, displacing material from the larger diameter end of the piece into a recess in the supporting face of the anvil member, and then while the piece is firmly held between the anvil member and the punch and maintained against lateral shifting by the nose of the punch in said recess and the displaced material in the recess in the face of the anvil member trimming the longitudinal perimeter of the piece to expose clean material at the perimeter.

5. In a method of cleaning the longitudinal wall of a tapered ingot piece wherein one end of the piece is of an originally smaller diameter than the opposite end, placing the ingot piece with its larger end on an anvil member having a diameter substantially the same as the diameter of the larger end of the piece, driving a shallow-

taper generally frusto-conical punch nose having a substantial diameter relative to the diameter of the ingot centrally into the smaller diameter end of the piece and thereby pressing a shallow complementary frusto-conical depression into said smaller diameter end and thus displacing material of the piece from the smaller diameter end thereof downwardly and laterally and thereby bulging the longitudinal perimeter of the piece into substantially uniform shape and eliminating the taper thereof, and trimming off the bulged perimeter of the piece to expose clean material on the perimeter of the piece.

References Cited in the file of this patent

UNITED STATES PATENTS

|    |           |                  |               |
|----|-----------|------------------|---------------|
| 15 | 635,097   | Heinle           | Oct. 17, 1899 |
|    | 1,186,055 | White            | June 6, 1916  |
|    | 1,396,281 | Paque            | Nov. 8, 1921  |
|    | 1,434,190 | Bird             | Oct. 31, 1922 |
| 20 | 1,456,597 | Hughes           | May 29, 1923  |
|    | 1,486,365 | Cummings         | Mar. 11, 1924 |
|    | 1,672,999 | Eyermann         | June 12, 1928 |
|    | 1,714,661 | Crawford et al.  | May 28, 1929  |
|    | 2,106,647 | Neck             | Jan. 25, 1938 |
| 25 | 2,406,062 | Cornell          | Aug. 20, 1946 |
|    | 2,502,737 | Meley et al.     | Apr. 4, 1950  |
|    | 2,698,951 | Van Haandel      | Jan. 11, 1955 |
|    | 2,821,016 | Dickson          | Jan. 28, 1958 |
|    | 2,869,432 | Sedlaczek et al. | Jan. 20, 1959 |

FOREIGN PATENTS

|         |               |               |
|---------|---------------|---------------|
| 26,113  | Great Britain | Nov. 11, 1910 |
| 212,331 | Great Britain | Mar. 13, 1924 |

OTHER REFERENCES

35 Adler: Abst. of application Ser. No. 722,180, Feb. 14, 1950, vol. 631, page 584 O.G. 78-63.